

June 27, 1939.

H. R. GUNDLACH

2,163,678

COLORED ROOFING GRANULE

Filed July 1, 1936

*Fig. 1*



*Fig. 2*



*Inventor:*  
Henry R. Gundlach  
*By* *Gillmor, Mann & Cox Atty's.*

## UNITED STATES PATENT OFFICE

2,163,678

## COLORED ROOFING GRANULE

Henry R. Gundlach, Baltimore, Md., assignor  
to Central Commercial Company, a corporation  
of Illinois

Application July 1, 1936, Serial No. 88,410

11 Claims. (Cl. 91—70)

This invention relates to roofing and more particularly to colored granules therefor and the method of coloring the granules.

One of the objects of the invention is the provision of new and improved means for attaching or securing color pigment to the surface of granules used on roofing material and the like.

Another object of the invention is the provision of new and improved means for color coating granules for use on roofing and the like, that is insoluble and when applied to the roofing material will resist, to a marked degree, the deleterious action of the weather including the actinic rays of the sun and will remain fixed on the roofing for an indefinite length of time.

A still further object of the invention is the provision of a new and improved method for retaining color pigment on granules and at the same time, providing a more or less roughened surface on the exterior of the colored granule whereby the granule may be easily retained on the roofing material by the weatherproof binder conventionally employed.

A further object of the invention is the provision of a new and improved colored granule that may be prepared at a minimum of expense; that will be firmly and permanently retained in position on the roofing material; that is insoluble; and, one in which the color is uniform and will remain fresh in appearance for an indefinite length of time.

Other and further objects and advantages of the invention will appear from the following description taken in connection with the accompanying drawing, in which:

Fig. 1 is a cross section of a roofing strip showing the granules in position thereon; and

Fig. 2 is a cross section, on an enlarged scale, of one of the granules.

It is common practice to artificially color granules for use on roofing material and the like; but, owing to the continued exposure of this material to all kinds of weather conditions, including the actinic rays of the sun, the color may fade and the retaining material may be caused to chip off or gradually dissolve, if not insoluble, or the binder for holding the granules to the roofing felt may be so adversely affected by the sun's rays or the binder dissolve to such an extent that not only the color pigment may gradually become loose and washed away but also the granules themselves may become loosened and later detached. This latter is especially true when the binder material for securing the pigment to the granule is more or less soluble or is transparent

and more especially if the granule itself is also transparent since the actinic rays of the sun will be transmitted through the granule thereby effecting photo-chemical changes in the asphalt and causing the same to deteriorate. In the use of certain binders that are more or less soluble, even though the solubility be fairly low, the exterior or exposed surfaces of the binder will, in time, dissolve to such an extent that the granules will become loose and later detached.

The present invention seeks to remedy these difficulties by the provision of a granule having color pigment secured to its exterior by a composition that is insoluble and that will not transmit the deleterious light rays to roofing material and to the binder employed for attaching the color pigment to the granules.

Referring now to the drawing, the reference character 10 designates a foundation roofing felt which has been impregnated with a bituminous or other water or weatherproof material as is usual in such constructions. The felt 10 is covered on one side by a binder of bituminous composition 11 of a rather high melting point, as asphalt or other suitable bituminous material. 25 Granules 12, having color pigment 13 secured to the surface thereof, are embedded in this material for protecting the felt. The granules may be of any suitable material, such as greenstone, trap rock, slate, quartz, or the like.

In the preparation of the granules, the material is first ground and then screened to the proper size in the usual or any suitable manner. After screening or sizing, the granules are given a coat 14 of a mixture, the base of which is a 35 soluble silicate such as sodium silicate. Sodium silicate alone may be employed, with or without color pigment, but if so, the sodium silicate is preferably fused onto the granules. Preferably, however, the sodium silicate is applied with or 40 without the color pigment together with a hardener or insolubilizer such as clay, calcium hydroxide, zinc oxide, or the like. This coat is applied in the conventional manner.

While this first coat is being applied, which 45 may be done in a rotary kiln by pouring a mixture of sodium silicate, water, and an insolubilizer or a solution of the sodium silicate alone, as the case may be, into the mass of granules and heating the mass for drying the same, the granules are continually agitated to prevent agglomeration. After the first coat has been applied by drying the same on the surface of the granules by application of heat or by subjecting the coat to sufficient heat to 50 55

fuse the sodium silicate, as the case may be, the second coat is applied.

The amount of sodium silicate of the first coat may vary within rather wide limits and the subsequent treatment may vary considerably. It is immaterial how the coat is applied or what type or amount of sodium silicate is employed.

The following formulas for the first coat will indicate the proportions of the ingredients and are given by way of example only:

**FIRST COAT**

**Formula No. 1**

|                  | Pounds |
|------------------|--------|
| 15 Lawrence clay | 25-40  |
| Pigment          | 0-10   |
| Sodium silicate  | 20-40  |
| Water            | 10-22  |

Mix A and B together and apply to one ton granules, dry in carbon dioxide free air and heat to 600°-1100° F. for 10-30 minutes, in order that clay and silicate react.

**Formula No. 2**

|                      | Pounds |
|----------------------|--------|
| 25 Calcium hydroxide | 20-25  |
| Zinc oxide           | 4-6    |
| Pigment              | 0-10   |
| Sodium silicate      | 50-70  |
| Water                | 20-30  |

Dry as in above first coat and heat to 400°-600° F. for 10-30 minutes. If desired, the sodium silicate may be first applied and dried and the insolubilizing composition applied to the heated granules.

After the first coat has been applied and has been dried on the granule, a second coat is now applied which is opaque and will form a more or less rough surface on the exterior of the granule.

This second coat is a reaction product of phosphoric acid on a silicate or on calcareous, aluminous or siliceous material, or on any two of these materials. The reaction products of phosphoric acid and compounds of one or more of the common metals of Groups III, IV, VII or VIII of the periodic classification of the elements that are capable for forming sesqui-oxides may also be employed. The compounds of these elements most suitable are the oxides, hydroxides or carbonates thereof. The compounds of the more common metals of Group II of the periodic classification of the elements as the oxides, hydroxides or carbonates may also be used with satisfactory results. Satisfactory results are obtained by calcining a mixture of clay, lime and siliceous material, or any two of these materials, grinding the calcined material and then mixing the ground material with the granules and color pigment and adding phosphoric acid.

The following formulas are given by way of example only, as compositions or mixtures that may be sintered or calcined and reduced to form what may be termed cement powder for reacting with phosphoric acid to form a binder for attaching the color pigment to the surfaces of the granules:

**Formula No. 1**

|                   | Per cent |
|-------------------|----------|
| Clay              | 72       |
| Calcium carbonate | 28       |

**Formula No. 2**

|                   | Per cent |
|-------------------|----------|
| Clay              | 69.8     |
| Calcium carbonate | 27.2     |
| Cryolite          | 3.0      |

**Formula No. 3**

|                   | Per cent |
|-------------------|----------|
| Calcium carbonate | 48.0     |
| Aluminum oxide    | 52.0     |

**Formula No. 4**

|                        | Per cent |
|------------------------|----------|
| Sodium silico-fluoride | 36.4     |
| Calcium fluoride       | 5.1      |
| Aluminum oxide         | 32.4     |
| Silica                 | 26.1     |

**Formula No. 5**

|                   | Per cent |
|-------------------|----------|
| Calcium carbonate | 16 to 17 |
| China clay        | 83 to 84 |

**SECOND COAT**

After the granules have been treated with the first coat including the insolubilizing composition, the second coat is then applied.

The following formulas have been found to give satisfactory results for the second coat. These formulas are given by way of example only:

**Formula No. 1**

|                                                         | Pounds |
|---------------------------------------------------------|--------|
| Cement powder                                           | 12     |
| Pigment                                                 | 4-25   |
| Filler, if desired, possibly as much as 15 lbs.—silica. | 30     |
| Phosphoric acid, 75%                                    | 32.4   |
| Zinc oxide                                              | 1.2    |
| Water                                                   | 22.4   |

**Formula No. 2**

|                      | Pounds |
|----------------------|--------|
| Cement powder        | 9      |
| Pigment              | 4-20   |
| Filler, if desired.  |        |
| Phosphoric acid, 75% | 22.1   |
| Zinc oxide           | .9     |
| Water                | 26.0   |

The first coat is soluble to a certain extent but when covered by the second coat containing insoluble phosphate, there appears to be a reaction between the elements of the two coats. At any rate, the resultant material is more nearly insoluble than the material of either coat alone. This is considered an important feature of the invention. This method of coating the granules also reduces the tendency to bloom or effloresce. The color too appears to be more vivid, which is probably due to a better distribution of color. Furthermore, the second coat being opaque will prevent the passage of actinic rays therethrough and being more or less rough on its surface, the bituminous binder will firmly anchor the granule to the roofing material.

It is also common practice to employ frits or other igneous binders for attaching color pigment to the surface of the granules. Frit is applied in a single or a plurality of coats and the color pigment may be in either or both coats. In any event, the exterior of the colored granule will be smooth and glassy and consequently, the granules will not be sufficiently firmly held by the bituminous binder of the roofing material to prevent their becoming loosened by the mechanical action of hail, rain, wind, and the like. Furthermore, since the frit is more or less transparent, and if used on transparent or translucent granules, the sun's rays will pass through the same and injuriously effect the adjacent adhering binder, whereby the granules will loosen and become displaced.

This difficulty is overcome by applying an outer phosphate coat or binder material as previously described.

In this method, as in the method previously described, the phosphate coat or binder material is applied in the same manner described before and the color pigment may be in the outer or phosphate coat or in both or all coats, as desired. The rough surface of the phosphate coat will constitute means for anchoring the granule to the roofing material inasmuch as the asphaltic or bituminous binder will more firmly adhere to a rough surface than to a smooth one.

Instead of employing an outer coat composed of the reaction product of phosphoric acid, any composition or mixture that will form a cementitious waterproof cement or binder and that is more or less opaque and has rough exterior may also be employed.

20 It is thought from the foregoing taken in connection with the accompanying drawing that the method and process of my invention will be apparent to those skilled in the art, and that changes may be made without departing from the spirit and scope of the appended claims.

I claim as my invention:

1. A method of coloring granules of mineral matter for use on composition roofing comprising coating the granule with a first-coat composition comprising a sodium silicate solution and an insolubilizer, drying the same on the granule and then applying a cementitious substantially insoluble material on said first coat, said material including phosphoric acid as the major ingredient aside from water and color pigment to the surface of the coated granule, and then drying the second coat.

2. A method of coloring roofing granules which comprises coating the granule with a soluble silicate and a hydroxide of the calcium group, dehydrating the silicate, and then covering the coated granule with a second coat comprising an insoluble phosphate having color pigment incorporated therein, the phosphate constituting the principal ingredient of the coating.

3. Composition roofing comprising, a sheet of roofing material impregnated with a bituminous compound and having colored granules secured to one surface thereof, each granule enveloped in a coat of material including a soluble silicate fused thereon, and color pigment secured to the surface of said coat by a binder formed by the reaction products of a mixture of ground calcareous and siliceous material and phosphoric acid.

4. An artificially colored granule for use on composition roofing comprising a granule of mineral matter having an inner coat of sodium silicate and an outer coat comprising color pigment secured to the surface of said inner coat by the reaction product of a silicate and a radical of phosphoric acid as the major ingredient by weight, aside from the water.

5. The method of coloring granules which comprises fusing an igneous coat including a soluble silicate on the surface of the granule and then securing color pigment to the surface of the coated granule by a cement formed by the reaction product of calcined calcareous, aluminum and siliceous materials and phosphoric acid.

6. The method of coloring granules which comprises coating the granule with sodium silicate and an insolubilizing agent, drying the mass, and then coating the granule with a second coat comprising color pigment, a composition including a

compound of one of the common metals of Groups III, IV, VII or VIII of the periodic classification of the elements capable of forming a sesqui-oxide and phosphoric acid.

7. A method of coloring granules for use on composition roofing which comprises covering the granules with a coat formed from a mixture of:

|                 | Pounds  |
|-----------------|---------|
| Lawrence clay   | 25-40   |
| Color pigment   | 0-10 10 |
| Sodium silicate | 20-40   |
| Water           | 10-22   |

for each ton of granules, drying the mass in carbon dioxide free air and heating from 600° F. to 15 1100° F. and then coat the granules with a mixture comprising a color pigment and an insoluble phosphate.

8. A method of coloring granules for use on composition roofing which comprises covering the granules with a coat formed from a mixture of:

|                   | Pounds  |
|-------------------|---------|
| Calcium hydroxide | 20-25   |
| Zinc oxide        | 4-6     |
| Pigment           | 0-10 25 |
| Sodium silicate   | 50-70   |
| Water             | 20-30   |

dry the mass and heat from 400° F. to 600° F. for from 10 to 30 minutes and then applying a coat 30 of an insoluble phosphate.

9. A method of coloring granules for use on composition roofing which comprises coating the granules with a composition including sodium silicate, drying the same at a temperature between 600° F. and 1100° F. and then applying a coat containing a phosphate as the reaction product of phosphoric acid on sintered silicates and color pigment and finally drying the mass at a temperature between 400 to 600 degrees Fahrenheit.

10. A method of coloring granules which comprises coating the granules with the reaction product of a soluble silicate and an insolubilizer, drying the mass, and then applying a coat comprising color pigment and a cement formed by the reaction product of a calcined mixture of ground siliceous, aluminum material and phosphoric acid.

11. A method of coloring granules for use on composition roofing which comprises covering the granules with a coat formed from a mixture of:

|                 | Pounds   |
|-----------------|----------|
| Lawrence clay   | 25-40 55 |
| Color pigment   | 0-10     |
| Sodium silicate | 20-40    |
| Water           | 10-22    |

for each ton of granules, drying the mass in carbon dioxide free air and heating from 600° F. to 1100° F. and then applying a second coat formed from a mixture of:

|                       | Pounds          |
|-----------------------|-----------------|
| Cement powder         | 1 to 12         |
| Pigment               | 1 to 25 65      |
| Filler                | 0 to 15         |
| Silica                | 0 to 32.4       |
| Zinc oxide            | .9 to 1.2       |
| Phosphoric acid (75%) | 22.1 to 32.4 70 |

and water to form a cement, said cement powder comprising calcined mixture of ground clay and siliceous material.

HENRY R. GUNDLACH.